

## UNITED STATES PATENT OFFICE

GORDON PEACE, OF CAWNPORE, BRITISH INDIA, ASSIGNOR OF ONE-HALF TO THE  
BRITISH INDIA CORPORATION LIMITED, OF CAWNPORE, BRITISH INDIA, A CORPO-  
RATION

## RAPID VEGETABLE TANNING PROCESS

No Drawing. Application filed August 23, 1928, Serial No. 301,897, and in India December 8, 1927.

This invention relates to improved methods of tanning cow, ox and buffalo hides.

In the ordinary vegetable tanning processes if strong infusions of the tanning materials were used at the commencement of the process they would act too strongly on the surface of the skin under treatment, hardening and contracting it so that the subsequent tanning of the interior parts would be impeded. This is avoided in the methods ordinarily employed by the use at first of very weak infusions. In the case of sole leather the tanning process may require from three to twelve months for completion. The time taken in tanning is now however often shortened by "drumming" and other processes of agitation, assisted very often by the use of strong extract liquors.

The present invention has for its object to 20 prepare the hides in such a state that they may be rapidly penetrated by the tanning liquors and the tanning completed in a month or less in the case of heavy hides such as sole hides, and in a week or two depending upon 25 the thickness in the case of light hides such as cow hides for upper leather, without the use of drumming or the concentrated extract liquors hitherto employed to shorten the tanning process being necessary.

30 This is effected by means of the present invention according to which the hides, after liming and preparation for tanning in the ordinary way, are first subjected to the action of an appropriate pickling solution until 35 they are completely delimed and pickled through, whereafter the pickled hides are subjected to the action of a depickling solution until they are depickled and brought to a degree of acidity represented by a hydrogen-ion concentration of between about 40 pH 3.5 and pH 5.0 that they can be acted upon by the tanning liquor in a comparatively short time, the hides so treated being then subjected to treatment with the 45 desired vegetable tanning liquor of the requisite strength and in such manner as to effect their rapid tanning. The depickled hides may, if desired, be washed before subjecting them to the tanning operation.

50 For the production of the best qualities of

leather it is essential to wash the hides after depickling so as to remove as much as possible of the soluble salts therefrom and render them soft and uniform throughout their substance, although for inferior grades of 55 leather the washing may be omitted. As an example of a suitable pickling solution there may be mentioned an aqueous solution of salt and sulphuric acid. The depickling solution should be so chosen as to have no ill effect 60 on the hide and must be such as to permit of the hide being brought to a degree of acidity represented by a hydrogen-ion concentration of between about pH 3.5 and pH 5.0; solutions of the sodium salts of most weak acids and 65 particularly sodium thiosulphate have been found to give excellent results, and by means of the latter the hides can be brought to a degree of acidity represented by a hydrogen-ion concentration of about pH 3.6 to 3.8. 70

Hides prepared in the manner previously mentioned may be rapidly tanned by any of the methods ordinarily in use, the use of such weak infusions as hitherto employed at the commencement of the operation being unnecessary and the tanning of the hides if desired being started in the stronger liquors. It is desirable to maintain the hydrogen-ion concentration of the tanning solution, as determined with the hydrogen electrode, at 75 80 least until the hides are struck through, between the required limits, for example of about pH 3.5 and pH 5.0, depending on the degree of firmness required in the finished leather and on the tanning materials used in 85 the preparation of the tan liquors.

An example of the treatment of sole leather by the improved process according to the present invention is as follows:—The limed 90 unhaired and fleshed hides prepared in the usual manner are suspended in a pickle consisting of 80 grams of salt and 7.5 grams of sulphuric acid per litre of water until the 95 hides are completely delimed and are in a uniform state throughout their substance. The hides are then suspended in a 10-15 per cent solution of sodium thiosulphate until they are depickled and brought to a degree of acidity represented by a hydrogen-ion concentration of between about pH 3.6 and 100

pH 3.8 whereafter they are washed for several hours in running water. They are then ready for tanning. In the case of a liquor prepared from the following materials, babul bark 9 parts, myrobalans 1 part and wattle bark 1.5 parts, they may be suspended at once in a liquor of 60 degree barkometer strength, and provided the strength is maintained a medium thickness hide will be tanned in about 14 days. The actual tanning process used may be varied through wide limits depending on the tanning materials used and weak liquors may be given if desired, but it is necessary if a well tanned leather is required to increase rapidly the strength of the liquor if the tanning is to be completed in a month or less. For example the process just given may be varied by introducing the hides into a 40 degree barkometer liquor for two days, a 50 degree liquor being given on the third day, and a 60 degree liquor on the 4th or 5th day, the strength of this liquor being maintained until the hides are tanned. As an example of another alternative method of carrying out the actual tanning process, the hides may be treated in an 8 degree barkometer liquor for one day, a 17 degree liquor being given on the second day, a 22 degree liquor on the third day, a 25 degree liquor on the fourth day, and a 30 degree liquor on the fifth day, whereafter the hides are treated for 6 days in a 40 degree liquor, 6 days in a 45 degree liquor, 6 days in a 50 degree liquor, and one week in a 60 degree liquor. Except for the purposes of "loading" it is rarely necessary to use a stronger liquor than 60-65 degree barkometer.

For the softer leathers such as cow upper leathers the pickling, depickling and washing are carried out as previously described with regard to sole leather, except that they take place subsequent to the bating or other processes used normally for preparing the hides. The tanning is best carried out using weaker liquors than for sole leather and at the higher pH values. A medium thickness cow hide can be tanned in as little as 8 days or even less by suspension in a 10 degree liquor for one day, moving it forward daily into stronger liquors and finishing in a 30-40 degree liquor or alternatively the tanning may be started and carried out in a 30 or 40 degree barkometer liquor.

In both the examples given above, namely for the treatment of sole leather and also for the softer leathers, the step of washing the hides after depickling them can if desired be omitted, the hides in such case being taken straight from the depickling bath of sodium thiosulphate and subjected to treatment with the tanning liquor.

Other methods of pickling and depickling besides these mentioned can be employed, it being necessary of course to ensure that the particular pickling and depickling means

used are such that the hides are eventually left in a suitable condition, similar to that resulting from the particular pickling and depickling processes hereinbefore mentioned, to enable them to be rapidly tanned in a satisfactory manner. 70

It may be mentioned that the present process although it is primarily intended to enable the tanning process to be carried out in a much shorter period of time than was heretofore possible without the use of mechanical agitation and/or extract liquors of a high concentration which have constituted the chief means heretofore employed for shortening the tanning process, may nevertheless, if so desired, be employed in conjunction with one or other or both of the aforesaid means. 75

What I claim and desire to secure by Letters Patent of the United States is:— 85

1. A process for the rapid vegetable tanning of cow, ox and buffalo hides which consists in liming and preparing the hides for tanning in the ordinary way, then subjecting the hides to the action of a pickling solution until they are completely delimed and pickled through, subjecting the pickled hides to the action of a depickling solution comprising an aqueous solution of sodium thiosulphate until they are depickled only to such an extent that the hides are brought to a degree of acidity represented by a hydrogen-ion concentration of between about pH 3.5 and pH 5.0, and only thereafter subjecting the hides to treatment with a vegetable tanning liquor of the requisite strength so as to effect their rapid tanning. 95

2. A process for the rapid vegetable tanning of cow, ox and buffalo hides which consists in liming and preparing the hides for tanning in the ordinary way, then subjecting the hides to the action of a pickling solution until they are completely delimed and pickled through, subjecting the pickled hides to the action of a depickling solution comprising an aqueous solution of sodium thiosulphate until they are depickled only to such an extent that the hides are brought to a degree of acidity represented by a hydrogen-ion concentration of between about pH 3.5 and pH 5.0, removing the hides from the depickling solution and washing them, and thereafter subjecting the washed depickled hides to treatment with a vegetable tanning liquor of the requisite strength so as to effect their rapid tanning. 105

3. A process as in claim 1, in which the pickling solution comprises an aqueous solution of salt and sulphuric acid. 115

4. A process as in claim 2, in which the pickling solution comprises an aqueous solution of salt and sulphuric acid. 125

5. A process as in claim 1, in which the pickling solution comprises an aqueous solution of salt and sulphuric acid and in which 130

the tanning liquor is maintained at a degree of acidity represented by a hydrogen-ion concentration of between about pH 3.5 and pH 5.0 until the hides are struck through.

5 6. A process as in claim 2, in which the pickling solution comprises an aqueous solution of salt and sulphuric acid and in which the tanning liquor is maintained at a degree of acidity represented by a hydrogen-ion concentration of between about pH 3.5 and pH 5.0 until the hides are struck through.

10 GORDON PEACE.

15

20

25

30

35

40

45

50

55

60

65